# EUROPEAN PATENT SPECIFICATION

(11) **EP 0 566 814 B1**
(45) Date of publication and mention of the grant of the patent: **03.09.1997**
(21) Application number: 92830586.1
(22) Date of filing: 26.10.1992
(51) Int. Cl.: C22C 38/42, C22C 38/44

(54) **Superduplex stainless steel having high corrosion resistance and high yield strength in the solution annealed condition**
Rostfreies Superduplexstahl mit hohe Korrosionsbeständigkeit und hoher Dehngrenze in lösungsgeglühten Zustand
Acier inoxydable superduplex présentant une haute résistance à la corrosion et une limite élastique élevée à l'état recuit de mise en solution

(30) Priority: 24.04.1992 IT RM920309
(43) Date of publication of application: 27.10.1993
(73) Proprietor: FORONI S.p.A., I-21055 Gorla Minore (Varese) (IT)
(72) Inventor: Foroni,Luca, I-21055 Gorla Minore (Va) (IT)

(56) References cited:
- EP-A- 0 360 143
- GB-A- 2 160 221
- GB-A- 2 203 680
- US-A- 4 816 085

## Description

The Austenitic/Ferritic stainless steels presently on the market are those reported in the ASTM A790 specification with the addition of the Zeron 100, equivalent to UNS S32760, which is not yet included in the ASTM specification.

The steel grades which are mainly requested for the oil field applications are the UNS S32750 and UNS S32760.

There are however many other kind of steels which can be included in the same class and which are listed and described in the following publications :
- Superduplex Stainless Steel : Structure and Properties. by J. Charles
- Superduplex Stainless Steel : Structure and Properties. by J. Charles
- The Corrosion Resistance of Duplex Stainless Steel. by S. Bernhardsson

The invention concerns the production of austenitic-ferritic stainless steel of the superduplex class, manufactured by electrical arc melting and A.O.D. refining.

The A.O.D. refining allows a deep deoxydation and desulphurization of the steel as well as to reach the required chemical composition in a repeatable way.

The analytical balancing of the alloying elements Cr, Mo, W, Cu and N is very important for obtaining the mechanical properties and the corrosion resistance on hot forged and/or rolled products in the solu tion annealed condition.

Our invention has taken advantage of the combined action of Mo, W, Cu, N which allows to reach a yield strength value higher than 620 MPa (90,000 PSI) as well as a generalized resistance to the stress corrosion, to the pitting and crevice corrosions.

The optimized chemical composition is the following :
(weight in percent)

| | |
|---|---|
| C | 0.025 max |
| Mn | 0.80 max |
| Si | 0.80 max |
| Cr | 24 - 26 |
| Ni | 6.5 - 8.0 |
| Mo | 3.0 - 4.0 |
| S | 0.002 max |
| P | 0.025 max |
| Cu | 1.2 - 2.0 |
| W | 0.80 - 1.2 |
| N | 0.23 - 0.33 |
| Fe | balance |

The ferrite on the product solution annealed at the temperature of 1070 - 1100°C is 40 - 55%

Pitting index = Cr + 3.3 Mo + 16 N > 42

1. Mechanical characteristics of the product solution annealed at 1080 °C :

| | | Room Temp. | 80°C | 150°C |
|---|---|---|---|---|
| Rs 0.2 MPa (KSI) | | 630 (91) | 550 (80) | 480 (70) |
| R MPa (KSI) | | 865 (125) | 800 (116) | 750 (110) |
| A % | | 40 | | |
| HB | | 270 | | |
| | °C | -45 | -65 | -100 |
| KV | | | | |
| | Joule | 300 | 144 | 38 |

2. Comparisons with other steels of the same class on the basis of the corrosion resistance :
2.1 Chemical analysis of steel (A = Steel subject of the invention)

| | Cr | Ni | Mo | Cu | W | N |
|---|---|---|---|---|---|---|
| A) | 25.5 | 7.4 | 3.9 | 1.7 | 0.9 | 0.27 |
| B) | 25.5 | 7.1 | 3.6 | 0.7 | 0.7 | 0.26 |
| C) | 25.4 | 7.0 | 3.6 | 0.2 | --- | 0.28 |

2.2 Pitting corrosion resistance (ASTM G48) at 50°C - 24 h.

| | A | B | C |
|---|---|---|---|
| weight loss (g/m²) | 0.049 | 0.070 | 0.76 |
| N° of pitting/m² | 0 | 0 | 270 |
| Max pit depth (micron) | 0 | 0 | 100 |
| Critical Pitting Temp.(°C) | 80 | 60 | 50 |

2.3 Corrosion resistance in 5% Na Cl at PH = 4 - 6 at 600 mV :

| | A | B | C |
|---|---|---|---|
| CPT (°C) | 80 | 72 | 63 |

2.4 Crevice corrosion resistance (ASTM G78 modified) 100 days .
- Environment :: Aerated sea water containing 20,000 ppm cloride plus 2 ppm residual chlorine with occasional shock dosing up to 10 ppm chlorine ar 35°C

| | A | B | C |
|---|---|---|---|
| N° of crevice (min/max) | Absent | 1 / 3 | Traces |

2.5 Sulfide Stress Cracking Resistance of the steel object of the invention (NACE TM-01-77) at 80°C - 760 h :
Applied load = 550 MPa no cracking

## Claims

1. Alloy having the chemical composition (in percent by weight) :
| | |
|---|---|
| C | 0.025 max |
| Mn | 0.80 max |
| Si | 0.80 max |
| Cr | 24 - 26 |
| Ni | 6.5 - 8.0 |
| Mo | 3.0 - 4.0 |
| S | 0.002 max |
| P | 0.025 max |
| Cu | 1.2 - 2.0 |
| W | 0.8 - 1.2 |
| N | 0.23 - 0.33 |
| Fe | balance |
Pitting Index = Cr + 3.3 Mo + 16 N > 42
Balanced chemical composition to obtain after solution heat treatment at 1070-1100°C an alfa Ferrite of 40 - 60%.

2. Alloy according to claim 1, characterized in that the content of C is 0.01 - 0.02%.

3. Alloy according to claim 1, characterized in that the content of Si is 0.35 - 0.60%.

4. Alloy according to claim 1, characterized in that the content of Ni is 7.0 - 7.5%.

5. Alloy according to claim 1, characterized in that the content of Mo is 3.7 - 4.0%

6. Alloy according to claim 1, characterized in that the content of Cu is 1.6- 1.9%.

7. Alloy according to claim 1, characterized in that the content of W is 0.9- 1.1%.

8. Alloy according to claim 1, characterized in that the content of N is 0.25- 0.30%.

## Patentansprüche

1. Die chemische Zusammensetzung der Legierung lautet:
(in Gewichprozenten)
| | |
|---|---|
| C | 0.025 max |
| Mn | 0.80 max |
| Si | 0.80 max |
| Cr | 24 - 26 |
| Ni | 6.5 - 8.0 |
| Mo | 3.0 - 4.0 |
| S | 0.002 max |
| P | 0.025 max |
| Cu | 1.2 - 2.0 |
| W | 0.8 - 1.2 |
| N | 0.23 - 0.33 |
| Fe | Rest |
$\text{Grübchen-index = Cr + 3.3Mo + 16N > 42}$ Ausgewogene chemische Zusammensetzung, zu erzielen nach 1 ö sungsunterstürtzter Hitzbehandlung bei 1070-1100°C und Alpha-Ferrit zwischen 40-60%.

2. Legierung nach Patentanspruch 1: dadurch charakterisiert, daß der C-Gehalt 0.01-0.02% beträgt

3. Legierung nach Patentanspruch 1; dadurch charakterisiert, daß der Si-Gehalt 0.35-0.60% beträgt

4. Legierung nach Patentanspruch 1: dadurch charakterisiert, daß der Ni-Gehalt 7.0-7.5% beträgt

5. Legierung nach Patentanspruch 1: dadurch charakterisiert, daß der Mo-Gehalt 3.7-4.0% beträgt

6. Legierung nach Patentanspruch 1: dadurch charakterisiert, daß der Cu-Gehalt 1.6-1.9% beträgt

7. Legierung nach Patentanspruch 1: dadurch charakterisiert, daß der W-Gehalt 0.9-1.1% beträgt

8. Legierung nach Patentanspruch 1: dadurch charakterisiert, daß der N-Gehalt 0.25-0.30% beträgt

## Revendications

1. Alliage ayant la composition chimique suivante (pourcentage de poids):
| | |
|---|---|
| C | 0.025 max |
| Mn | 0.80 max |
| Si | 0.80 max |
| Cr | 24-26 |
| Ni | 6.5-8.0 |
| Mo | 3.0-4.0 |
| S | 0.002 max |
| P | 0.025 max |
| Cu | 1.2-2.0 |
| W | 0.80-1.2 |
| N | 0.23-0.33 |
| Fe | reste |
Index Pitting = Cr + 3.3 MO + 16 N > 42
Composition chimique équilibrée de façon à obtenir après hypertrempe à 1070-1100°C, de la Ferrtite alfa de 40-60%

2. Alliage suivant la condition requise 1, caractérisé par contenu de C de 0.01-0.02%;

3. Alliage suivant la condition requise 1, caractérisé par contenu de Si de 0.35-0.60%;

4. Alliage suivant la condition requise 1, caractérisé par contenu de Ni de 7.0-7.5%;

5. Alliage suivant la condition requise 1, caractérisé par contenu de Mo de 3.7-4.0%;

6. Alliage suivant la condition requise 1, caractérisé par contenu de Cu de 1.6-1.9%;

7. Alliage suivant la condition requise 1, caractérisé par contenu de W de 0.9-1.1%;

8. Alliage suivant la condition requise 1, caractérisé par contenu de N de 0.25-0.30%;
